



US011834760B2

(12) **United States Patent**  
**Woodruff et al.**

(10) **Patent No.:** **US 11,834,760 B2**  
(45) **Date of Patent:** **Dec. 5, 2023**

(54) **WRAPPABLE END FRAY RESISTANT WOVEN PROTECTIVE TEXTILE SLEEVE AND METHOD OF CONSTRUCTION THEREOF**

(71) Applicant: **FEDERAL-MOGUL POWERTRAIN LLC**, Mi, MI (US)

(72) Inventors: **Alexa A. Woodruff**, Bryn Mawr, PA (US); **Michael D. Knudson**, Mohnton, PA (US); **Tianqu Gao**, Exton, PA (US); **Cassie M. Malloy**, Exton, PA (US)

(73) Assignee: **Federal-Mogul Powertrain LLC**, Southfield, MI (US)

(\*) Notice: Subject to any disclaimer, the term of this patent is extended or adjusted under 35 U.S.C. 154(b) by 0 days.

(21) Appl. No.: **17/591,634**

(22) Filed: **Feb. 3, 2022**

(65) **Prior Publication Data**

US 2022/0154371 A1 May 19, 2022

**Related U.S. Application Data**

(62) Division of application No. 14/975,129, filed on Dec. 18, 2015, now Pat. No. 11,268,217.

(51) **Int. Cl.**

**D03D 1/00** (2006.01)

**D03D 3/02** (2006.01)

(Continued)

(52) **U.S. Cl.**

CPC ..... **D03D 1/0043** (2021.05); **D03D 3/02** (2013.01); **D03D 15/00** (2013.01); **D03D 15/283** (2021.01);

(Continued)

(58) **Field of Classification Search**

CPC .... D03D 1/0043; D03D 15/283; D03D 15/47; D03D 15/292; D03D 15/00; D03D 3/02;  
(Continued)

(56) **References Cited**

**U.S. PATENT DOCUMENTS**

6,003,565 A \* 12/1999 Whittier, II ..... D03D 15/283  
139/420 A

**OTHER PUBLICATIONS**

Polymer Database, Melting Points of Polymers, accessed online Nov. 21, 2022.\*

\* cited by examiner

*Primary Examiner* — Camie S Thompson

(74) *Attorney, Agent, or Firm* — Robert L. Stearns;  
Dickinson Wright PLLC

(57) **ABSTRACT**

An end fray resistant textile sleeve includes an elongate wall having warp yarns extending generally parallel to a longitudinal central axis of the sleeve and fill yarns extending circumferentially about the sleeve. The warp yarns include at least two different types of yarns, with one of the types of warp yarns including activateable yarns and another of the types of yarns including non-activateable yarns. The activateable yarns can be provided as being activateable by at least one of heat, fluid and/or pressure, such that upon being activated, the yarns are caused to bond with the adjacent non-activateable warp yarns, as well as with the weft yarns with which they make contact. As such, the activateable yarns, upon being activated, become fixed with abutting warp yarns and weft yarns, thereby inhibiting end fray from resulting during a subsequent cold-cutting operation as well as in use.

**7 Claims, 3 Drawing Sheets**



(51) **Int. Cl.**  
*H01B 7/00* (2006.01)  
*H01B 7/18* (2006.01)  
*D03D 15/587* (2021.01)  
*D03D 15/283* (2021.01)  
*D03D 15/00* (2021.01)  
*D03D 15/292* (2021.01)  
*D03D 15/47* (2021.01)

(52) **U.S. Cl.**  
CPC ..... *D03D 15/292* (2021.01); *D03D 15/47* (2021.01); *D03D 15/587* (2021.01); *H01B 7/0045* (2013.01); *H01B 7/185* (2013.01);  
*D10B 2401/04* (2013.01); *D10B 2401/041* (2013.01)

(58) **Field of Classification Search**

CPC ..... D03D 15/587; D10B 2401/04; D10B 2401/041; H01B 7/0045; H01B 7/185  
USPC ..... 385/102; 138/123; 428/36.1, 36.3, 35.1;  
442/302, 192, 197, 208, 209; 139/419,  
139/390, 388

See application file for complete search history.

FIG. 1A



FIG. 1B



FIG. 2





FIG. 4A



FIG. 4B



FIG. 4C



FIG. 4D



FIG. 4E



## 1

**WRAPPABLE END FRAY RESISTANT  
WOVEN PROTECTIVE TEXTILE SLEEVE  
AND METHOD OF CONSTRUCTION  
THEREOF**

**CROSS-REFERENCE TO RELATED  
APPLICATION**

This U.S. Divisional Patent Application claims priority to U.S. Utility patent application Ser. No. 14/975,129, filed Dec. 18, 2015, the entire contents of which are incorporated herein by reference.

**BACKGROUND OF THE INVENTION**

1. Technical Field

This invention relates generally to protective sleeves for elongate members, and more particularly to woven textile sleeves.

2. Related Art

Elongate members, such as wires or wire harnesses, are commonly protected against abrasion and contamination by wrappable textile sleeves. It is known to construct wrappable textile sleeves from woven yarns. In order to form the desired sleeve length, and to avoid fraying the ends of the sleeve, it is known to use lasers, ultrasonic cutting devices, and the like, which melt the material of the sleeve wall during the cutting process, thereby reducing the likelihood of causing the material of the sleeve wall to fray. In addition, it is known to apply a chemical coating agent to the sleeve wall after forming the sleeve wall and prior to cutting the sleeve wall to reduce the likelihood of fraying the material of the sleeve wall during the cutting process. Although the aforementioned mechanisms can be effective in reducing the likelihood of fraying the material of the sleeve wall, they require specialized cutting devices or processes, and thus, they come at an added cost.

**SUMMARY OF THE INVENTION**

An end fray resistant textile sleeve for protecting elongate members is provided. The sleeve includes an elongate wall having warp yarns extending generally parallel to a longitudinal central axis of the sleeve and fill yarns extending circumferentially about the sleeve. The warp yarns and the fill yarns are woven in an overlying and underlying weave pattern with one another. The warp yarns include at least two different types of yarns, with one of the types of warp yarns including activateable yarns and another of the types of yarns including non-activateable yarns. The activateable yarns can be provided as being activateable by at least one of heat, fluid and/or pressure, such that upon being activated, the yarns are caused to bond with the adjacent non-activateable yarns, as well as with the weft yarns with which they make contact. As such, the activateable yarns, upon being activated, become fixed with the aforementioned non-activateable warp yarns and weft yarns, thereby inhibiting end fray from resulting during a subsequent cold-cutting operation that is performed to cut the sleeve to length as well as in use.

In accordance with another aspect of the invention, the activateable yarns can be provided as monofilaments and/or multifilaments.

## 2

In accordance with another aspect of the invention, the activateable yarns can be provided as monofilaments and/or multifilaments of non-activateable material coated with an activateable material.

5 In accordance with another aspect of the invention, the activateable yarns can be provided as bicomponent monofilaments having a central core of a material having a first melt temperature and an outer sheath of a material having a second melt temperature, wherein the first melt temperature is higher than the second melt temperature.

10 In accordance with another aspect of the invention, the activateable yarns can be provided as entangled yarns including non-activateable material entangled with activateable material.

15 In accordance with another aspect of the invention, the activateable yarns can be provided as a non-activateable monofilament or multifilament yarn twisted or served with an activateable monofilament or multifilament yarn.

20 In accordance with another aspect of the invention, the overlying and underlying weave pattern is formed as one of a plain, rib, basket or twill weave pattern.

25 In accordance with another aspect of the invention, the fill yarns can be provided at least in part as multifilaments to provide the wall with enhanced protection coverage.

30 In accordance with another aspect of the invention, the wall can be formed as a wrappable wall having opposite edges extending generally parallel to the central longitudinal axis wherein the opposite edges are brought into overlapping relation with one another.

35 In accordance with another aspect of the invention, the fill yarns can be provided at least in part as heat-set yarns to bias the opposite edges into overlapping relation with one another.

40 In accordance with another aspect of the invention, the wall can be formed as a seamless, circumferentially continuous wall.

45 In accordance with another aspect of the invention, a method of constructing an end fray resistant textile sleeve for protecting elongate members is provided. The method includes forming an elongate wall by weaving warp yarns and fill yarns with one another in an overlying and underlying weave pattern. The method further includes providing the warp yarns including at least two different types of yarns, with one of the types of warp yarns being activateable yarns and another of the types of warp yarns including non-activateable yarns. The method further includes activating the activateable yarns via application of at least one of heat, fluid and/or pressure, such that upon being activated, the activated yarns are caused to bond with the adjacent non-activateable yarns, as well as with the weft yarns with which they make contact. As such, the activated warp yarns become fixed with the aforementioned non-activateable warp yarns and weft yarns, thereby inhibiting weft yarns falling out opposite ends of the sleeve during a subsequent cold-cutting operation that is 55 performed to cut the sleeve to length as well as in use.

50 In accordance with another aspect of the invention, the method can further include providing the activateable warp yarns as monofilaments and/or multifilaments.

55 In accordance with another aspect of the invention, the method can further include providing the activateable warp yarns as bicomponent monofilaments having a central core of a material having a first melt temperature and an outer

60 In accordance with another aspect of the invention, the method can further include providing the activateable warp yarns as entangled yarns including non-activateable material entangled with an activateable material and/or multifilaments of non-activateable material coated with an activateable material.

65 In accordance with another aspect of the invention, the method can further include providing the activateable warp yarns as a non-activateable monofilament or multifilament yarn twisted or served with an activateable monofilament or multifilament yarn.

sheath of a material having a second melt temperature, wherein the first melt temperature is higher than the second melt temperature.

In accordance with another aspect of the invention, the method can further include providing the activateable warp yarns as entangled yarns including non-activateable material entangled with activateable material.

In accordance with another aspect of the invention, the method can further include providing the activateable warp yarns as a non-activateable monofilament or multifilament yarn twisted or served with an activateable monofilament or multifilament yarn.

In accordance with another aspect of the invention, the method can further include forming the weave pattern as one of a plain, rib, basket or twill weave pattern.

In accordance with another aspect of the invention, the method can further include providing the fill yarns at least in part as multifilaments to provide the wall with enhanced protection coverage.

In accordance with another aspect of the invention, the method can further include forming the wall as a wrappable wall having opposite edges extending generally parallel to the central longitudinal axis and bringing the opposite edges into overlapping relation with one another.

In accordance with another aspect of the invention, the method can further include heat-setting at least some of the fill yarns to bias the opposite edges into overlapping relation with one another.

In accordance with another aspect of the invention, the method can further include forming the wall as a seamless, circumferentially continuous wall.

#### BRIEF DESCRIPTION OF THE DRAWINGS

These and other aspects, features and advantages of the invention will become readily apparent when considered in connection with the following detailed description of presently preferred embodiments and best mode, appended claims and accompanying drawings, in which:

FIG. 1A is a schematic perspective view of a protective sleeve constructed in accordance with one presently preferred embodiment shown protecting an elongate member;

FIG. 1B is a schematic perspective view of a protective sleeve constructed in accordance with another presently preferred embodiment shown protecting an elongate member;

FIG. 2 is an enlarged partial plan view of a wall of the sleeves of FIGS. 1A and 1B constructed in accordance with one aspect of the invention;

FIGS. 3A-3C are schematic plan views illustrating different walls of the sleeves of FIGS. 1A and 1B in accordance with different aspects of the invention; and

FIGS. 4A-4E are schematic plan views illustrating different activateable warp yarns of the sleeves of FIGS. 1A and 1B in accordance with different aspects of the invention.

#### DETAILED DESCRIPTION OF PRESENTLY PREFERRED EMBODIMENTS

Referring in more detail to the drawings, FIGS. 1A and 1B illustrate a end fray resistant textile sleeves, with the sleeve 10 of FIG. 1A being an "open" sleeve and the sleeve 10' being a "closed" sleeve, discussed in more detail hereafter, wherein the same reference numerals are used to identify like features for both sleeves 10, 10'. The sleeves 10, 10' will be referred to hereafter as sleeve, in singular fashion, though it will be made clear by the use of unprimed and primed

reference numerals that both sleeves 10, 10' are being discussed. This said, it is to be recognized that all discussion hereafter applies to both sleeves 10, 10', unless expressly stated otherwise. The sleeve 10, 10' is particularly useful for protecting an elongate member 12 disposed in a cavity 13 of the sleeve 10, 10', such as conduits or wire harnesses, by way of example and without limitation. The sleeve 10, 10' has an elongate wall 14, 14' having warp yarns 16 extending generally parallel to a longitudinal central axis 17 of the sleeve 10, 10' and weft, also referred to as fill yarns 18 extending transversely to the warp yarns 16 and circumferentially about the wall 14, 14'. The warp yarns 16 and fill yarns 18 are woven with one another in an overlying and underlying desired weave pattern, such that they undulate over and under one another, such as in a plain, rib, basket or twill weave pattern, for example. The warp yarns 16 include at least two different types of yarns, with one of the types of warp yarns including activateable yarns 20 and another of the types of yarns including non-activateable yarns 22. The activateable yarns 20 can be provided as being activateable by at least one of heat, fluid and/or pressure, such that upon being activated, the yarns 20 are caused to bond with the adjacent non-activateable warp yarns 22, as well as with the weft yarns 18 with which they make contact. As such, the activateable yarns, upon being activated, become fixed with the aforementioned non-activateable warp yarns 22 and weft yarns 18, thereby inhibiting end fray from resulting during a subsequent cold-cutting operation that is performed to cut the sleeve 10 to length as well as in use.

The sleeve 10, 10' extends lengthwise along the longitudinal central axis 17 between opposite ends 24, 26. The sleeve 10, as indicated above, is "open", and thus, it has a lengthwise seam formed between opposite sides 28, 30 that extend generally parallel to the longitudinal central axis 17 between the opposite ends 24, 26. The weft yarns 18 of the wall 14 can be provided, at least in part, as heat-settable yarns, such as mostly or entirely as monofilaments or multifilaments of a heat-formable material, such as poly(ethylene) terephthalate (PET) or poly(phenylene) sulfide (PPS), by way of example and without limitation, wherein the heat-settable weft yarns 18 can be heat-set to bias the opposite sides 28, 30 into overlapping relation with one another. In use, during installation, the opposite sides 28, 30 can be readily spread apart from one another to facilitate installing the elongate member 12 therein, and then the sides 28, 30 can be released to allow the sides 28, 30 to automatically return to their overlapping relation, thus, providing protection about the entire circumference of the elongate member 12. In addition to the heat-settable weft yarns, it should be recognized that non-heat-settable weft yarns 18 can also be incorporated in the wall 14 of the sleeve 10, as desired for the intended application.

The sleeve 10', as indicated above, is "closed", and thus, it has a circumferentially continuous, seamless wall 14' extending about the cavity 13 between the opposite ends 24, 26. It should be recognized that the weft yarns 18 of the wall 14' can be provided as discussed above for the wall 14, thereby allowing the wall 14' to be heat-set to facilitate maintaining a generally round configuration of the cavity 13. Other than being closed, the sleeve 10' and its material content can be the same as that for the open sleeve 10.

As evidenced in the various embodiments illustrated in the drawings, the activatable warp yarns 20 can be woven in different ways to provide the sleeve 10, 10' with the physical attributes desired. For example, as shown in FIG. 2, wherein a portion of an open wall 14 of the sleeve 10 is illustrated, the activatable warp yarns 20 are shown as being woven as

individual, single yarns in circumferentially spaced relation from one another. The individual activatable warp yarns **20** are spaced circumferentially from one another by intervening non-activateable warp yarns **22**. In the embodiment shown, the wall **14** has a ratio of activatable to non-activateable warp yarns of about 1:6. It should be recognized that this pattern and ratio is equally applicable to the wall **14'** of the sleeve **10'**. Upon being woven, the activatable warp yarns **20** are activated, such as via heat, pressure and/or fluid, thereby causing the activated warp yarns **20** to bond with the adjacent, abutting non-activateable warp yarns **22** as well as with the weft yarns **18**. As such, during a subsequent cutting operation, such as a cold cutting operation, the weft yarns **18** adjacent the ends **24**, **26** of the cut sleeve **10**, **10'** are inhibited from unraveling and fraying due to being bonded with the activated warp yarns **20**.

In FIGS. 3A-3C, further embodiments illustrating plan views of different weave patterns of the activatable warp yarns are shown, with it being understood that the patterns of FIGS. 3A and 3B are schematic plan view representations for both open and closed sleeves **10**, **10'**, while FIG. 3C is a schematic plan view representation of a minimum location of activatable warp yarn **20** for the open sleeve **10** along its opposites sides **28**, **30**. In FIG. 3A, a relatively increased presence of the activatable warp yarn **20** relative to the non-activateable warp yarn **22** is shown for the sleeve **10**, **10'**. The ratio of activatable warp yarn **20** to the non-activateable warp yarn **22** is shown as being about 1:1. In the embodiment illustrated, the activatable warp yarn **20** is shown as being arranged in a plurality of bundles **32**. Each bundle **32** includes a plurality of activated warp yarns **20**, shown by way of example and without limitation as being four, arranged in side-by-side abutting relation with one another, with each bundle **32** being spaced circumferentially from one another by a plurality of the non-activateable warp yarns **22**, shown by way of example and without limitation as being four. It should be recognized, that although not shown for simplicity, that weft yarns **18** are woven with the warp yarns **16**, wherein the individual warp and weft yarns **16**, **18** can be woven via any suitable weave pattern, such as a plain weave pattern, by way of example and without limitation, wherein abutting ones of the activated warp yarns **20** within the bundles **32** undulate over and under the weft yarns **18** out of phase with one another.

In FIG. 3B, a lesser presence of the activatable warp yarn **20** relative to the non-activateable warp yarn **22** is shown for the sleeve **10**, **10'** relative to the sleeve of FIG. 3A. The ratio of activatable warp yarn **20** to the non-activateable warp yarn **22** is shown as being about 1:3. In the embodiment illustrated, the activatable warp yarn **20** is shown as being arranged in a plurality of bundles **32**, similar to the bundles **32** shown in FIG. 3A; however, each bundle **32** only includes two activated warp yarns **20** arranged in side-by-side abutting relation with one another. Otherwise, the construction shown in FIG. 3B is similar to that discussed for FIG. 3A, wherein each bundle **32** is spaced circumferentially from one another by a plurality of the non-activateable warp yarns **22**, shown by way of example and without limitation as being 6.

In FIG. 3C, a minimized presence of the activatable warp yarn **20** relative to the non-activateable warp yarn **22** is shown for the open sleeve **10**. In the embodiment shown, bundles **32** of activatable warp yarns **20** are present only along the opposite sides **28**, **30**, wherein the bundles **32** can be formed having any desired number of activatable warp yarns **20**. It is contemplated that the activatable warp yarns **20** could be provided a single yarns along each side **28**, **30**;

however, this would provide a minimum amount of protection against end fray. The warp yarns **16** extending between the pair of bundles **32** are provided as non-activatable warp yarns **22**.

In FIGS. 4A-4E, a variety of different types of activatable warp yarns **20** are shown, wherein one or more of the different types of the activatable warp yarns **20** can be used in a single sleeve **10**, **10'**. In FIG. 4A, the activatable warp yarn **20** is shown as a multifilament yarn, wherein the multifilament includes at least some, or entirely heat-activateable, pressure activateable or fluid activateable material extending along its length. The multifilament can be formed of separate filaments intertwined with one another, or as an entangled member including activateable material entangled with non-activateable material, such as fibrous materials entangled with one another. In FIG. 4B, the activatable warp yarn **20** is shown as a monofilament, wherein the monofilament is comprised of heat-activateable, pressure activateable or fluid activateable material, such that upon being exposed to the appropriate heat, pressure or fluid source, the activatable warp yarn **20** becomes activated and bonds with the neighboring, abutting warp and weft yarns **16**, **18**. In FIG. 4C, the activatable warp yarn **20** is shown as a combination of yarns intertwined with one another, wherein the different yarns are shown as being twisted with one another, while in FIG. 4D the different yarns are shown as being served with one another. The different yarns combined with one another to form the activatable warp yarn **20** can include a non-activateable monofilament or multifilament yarn **34** twisted or served with an activateable monofilament or multifilament yarn **36**. In FIG. 4E, the activatable warp yarn **20** is shown as a bi-component monofilament, wherein the bicomponent monofilament includes a central core **38** of material having a first melt temperature and an outer sheath **40** of a material having a second melt temperature, wherein the first melt temperature is higher than the second melt temperature. In each of the aforementioned embodiments, the heat-activateable, pressure activateable or fluid activateable material, upon being exposed to the appropriate heat, pressure or fluid source, causes the activatable warp yarn **20** to become activated and bonded with the neighboring, abutting warp and weft yarns **16**, **18**. It is to be further understood that, in addition to the embodiments discussed above, it is contemplated that the activatable warp yarn **20** can be formed by coating an otherwise non-activateable yarn with an activateable coating or adhesive, whether the underlying non-activateable yarn material is a monofilament or multifilament.

Accordingly, a sleeve **10**, **10'** constructed in accordance with the invention, upon being woven, with the activatable warp yarns **20** having been activated and bonded with the neighboring abutting warp and weft yarns **16**, **18**, can be readily cold cut with minimal or no end fray resulting, thereby maximizing the useful life of the sleeve **10**, **10'** while also providing the sleeve **10**, **10'** with an aesthetically pleasing appearance.

Obviously, many modifications and variations of the present invention are possible in light of the above teachings. It is, therefore, to be understood that within the scope of the appended claims and any ultimately allowed claims, the invention may be practiced other than as specifically described and shown.

What is claimed is:

1. An end fray resistant textile sleeve for protecting elongate members, comprising:  
an elongate wall having warp yarns woven with weft yarns, said warp yarns extending lengthwise in gener-

ally parallel relation to a longitudinal central axis between opposite ends and said weft yarns extending generally transversely to said warp yarns, said warp yarns including a plurality of activateable warp yarns and a plurality of non-activateable warp yarns, said activateable warp yarns being activateable by at least one of heat, fluid and/or pressure, wherein said activateable warp yarns are activated and bonded with adjacent ones of said non-activateable warp yarns and with said weft yarns, at least some of said activated warp yarns being arranged in side-by-side, abutting relation with one another to form a plurality of bundled activated warp yarns, each of said bundled activated warp yarns being spaced circumferentially from one another by at least some of said non-activateable warp yarns.

2. The end fray resistant textile sleeve of claim 1 wherein the activated yarns are monofilaments.

3. The end fray resistant textile sleeve of claim 1 wherein the activated yarns are multifilaments.

4. The end fray resistant textile sleeve of claim 1 wherein said activateable yarns are bicomponent monofilaments having a central core of a material with a first melt temperature and an outer sheath of a material with a second melt temperature, wherein the first melt temperature is higher than the second melt temperature.

5. The end fray resistant textile sleeve of claim 1 wherein said activateable yarns are entangled yarns including non-activateable material entangled with activateable material.

6. The end fray resistant textile sleeve of claim 1 wherein said activateable yarns include a non-activateable monofilament or multifilament yarn twisted or served with an activateable monofilament or multifilament yarn.

15 7. The end fray resistant textile sleeve of claim 1 wherein said elongate wall is a seamless, circumferentially continuous wall.

\* \* \* \* \*